

# United States Patent [19]

Takemoto et al.

[11] 3,841,876

[45] Oct. 15, 1974

[54] **METHOD FOR MAKING A PHOSPHOR SCREEN OF A CATHODE-RAY TUBE**

[75] Inventors: **Takeo Takemoto; Yoshifumi Tomita, both of Mobara; Ichiro Ijichi; Sajiro Maeda, both of Toyohashi, all of Japan**

[73] Assignee: **Hitachi, Ltd., Tokyo, Japan**

[22] Filed: **June 19, 1973**

[21] Appl. No.: **371,569**

[30] **Foreign Application Priority Data**

June 30, 1972 Japan..... 47-65000

[52] U.S. Cl..... 96/36.1, 96/44, 96/45

[51] Int. Cl..... G03c 5/00

[58] **Field of Search** ..... 96/36.1, 36, 44, 45

[56] **References Cited**

UNITED STATES PATENTS

2,961,314 11/1960 Amdursky et al. 96/36.1

|           |         |                     |         |
|-----------|---------|---------------------|---------|
| 3,070,441 | 12/1962 | Schwartz.....       | 96/36.1 |
| 3,653,901 | 4/1972  | Etter.....          | 96/36.1 |
| 3,725,065 | 4/1973  | Fadner.....         | 96/36.1 |
| 3,775,116 | 11/1973 | Takemoto et al..... | 96/36.1 |

*Primary Examiner*—David Klein

*Assistant Examiner*—Edward C. Kimlin

*Attorney, Agent, or Firm*—Craig & Antonelli

[57] **ABSTRACT**

An improved method for making a phosphor screen of a cathode-ray tube in which light-exposed portions of a photosensitive layer of a shadow mask assembly are removed by washing the assembly with a detergent solution thereby providing definite light-transmissible holes in the photosensitive layer. Exposure of phosphor to light through the resulting shadow mask assembly provides a satisfactorily uniform pattern of phosphors.

**5 Claims, 3 Drawing Figures**

PATENTED OCT 15 1974

3,841,876

FIG. 1



FIG. 2



FIG. 3



## METHOD FOR MAKING A PHOSPHOR SCREEN OF A CATHODE-RAY TUBE

The present invention relates to a method for making a phosphor screen of a cathode-ray tube or more in particular to an improvement on the method for making a phosphor screen of a cathode-ray tube disclosed in French Pat. No. 7,143,315 corresponding to U.S. Patent Ser. No. 204,020, now U.S. Pat. No. 3,775,116, filed on Dec. 2, 1971.

In the method disclosed in the above-mentioned patent, light-exposed portions of a photosensitive layer are smaller in diameter than and in registration with the shadow mask openings, and the photosensitive layer lies on a transparent layer which is in turn formed on the shadow mask, thus constituting a shadow mask assembly to be used for forming phosphor dots smaller in diameter than the shadow mask openings on the inner surface of the cathode-ray tube. In the above-mentioned method, the light-exposed portions of the photosensitive layer remain unremoved over the shadow mask. This results in the lack of concentricity and/or roundness of the phosphor dots formed, often causing a resulting phosphor dot screen on the inner surface of the panel to undergo the serious problem of unevenness.

Further, in removing the photosensitive layer and transparent layer from the shadow mask in order to recover a shadow mask after the formation of the phosphor screen, the shadow mask is liable to be damaged by the presence of a bonding agent on the whole surface of the shadow mask.

An object of the present invention is to provide an improved method of forming a phosphor screen of a cathode-ray tube without the above-mentioned inconveniences.

The above and other objects, features and advantages will be made apparent from the detailed description taken in conjunction with the accompanying drawings, in which:

FIG. 1 is a sectional view showing the essential parts of an unfinished shadow mask assembly used in the method of the invention;

FIG. 2 is a diagram showing a sectional view of the manner in which the shadow mask assembly is mounted on the frame; and

FIG. 3 is a sectional view showing the essential parts of the shadow mask assembly for explaining an embodiment of the present invention.

According to the present invention, there is provided a method for making a phosphor screen of a cathode-ray tube comprising the steps of providing a transparent layer on that surface of a shadow mask which faces the phosphor screen within the cathode-ray tube, the shadow mask being carried by a supporting frame, the transparent layer being capable of attenuating light passing therethrough, providing a photosensitive layer on the transparent layer, exposing the photosensitive layer to light through the shadow mask and transparent layer to form light-exposed portions smaller in diameter than the shadow mask openings in the photosensitive layer, developing the light-exposed portions to form, in accordance with the shadow mask openings, a pattern of effective light-transmissible holes in the photosensitive layer thereby obtaining a shadow mask assembly, and forming a pattern of phosphors using the shadow mask assembly, wherein prior to the formation

of the phosphor pattern, the shadow mask assembly is washed with a detergent solution to remove the light-exposed portions of the photosensitive layer.

In FIGS. 1 to 3, same reference numerals designate similar members or elements.

First, a shadow mask 1 with openings of a predetermined diameter to be finally mounted on a cathode-ray tube is prepared, and a photosensitive sheet 2 consisting of a photosensitive layer 2a and a transparent layer 2b constituting a base film for the photosensitive layer 2a is closely attached, without being wrinkled, onto that surface 1a of the shadow mask 1 which is to face a phosphor screen. More in detail, the photosensitive sheet 2 is fixed on the shadow mask 1 at those portions which do not contribute to the formation of the phosphor screen by means of a bonding agent 3b put on the frame as shown in FIG. 2 or on the side face 3a of the shadow mask 1 engaged with the frame 3 or on both of the frame and the side face. This process requires to be followed for the reasons that in the event of the bonding agent being put substantially over the whole interface between the transparent layer 2b and the shadow mask 1, the transparent sheet 2 cannot be removed easily from the shadow mask 1 which may cause the shadow mask to be deformed, and further light is less easily passed through the shadow mask assembly at the later-described process of light-exposure.

If desired, wrinkles, if any, of the photosensitive sheet 2 may be removed by application of heat thereto even after the disposition of the photosensitive sheet 2. The photosensitive layer 2a may consist of polyvinyl chloride, natural rubber, synthetic rubber or the like which loses viscosity by photopolymerization in the presence of light or may consist of polyvinyl-carbazole which is accompanied by a change in its charged condition in the presence of light.

As the next step, the photosensitive sheet 2 is exposed to light with a high-pressure mercury lamp (not shown) through an opening 1c of the shadow mask 1 from the electron gun side 1b of the shadow mask 1 as indicated by the arrow in FIG. 1. In the process, assuming that the photosensitive layer consists of a material subject to photopolymerization, the temperature may be within the range from the room temperature to 90°C preferably 40° - 80°C in order to increase the photosensitivity of the photosensitive layer. 60°C is the most appropriate for the exposure. Light transmitted through the opening 1c of the shadow mask 1 reaches the photosensitive layer 2a through the transparent layer 2b, while being attenuated due to absorption and scattering in the transparent layer 2b. As a result, the light-exposed portion 4 of the photosensitive layer 2a in registration with the opening 1c of the shadow mask 1 is smaller in diameter than the opening of the shadow mask 1, as illustrated in FIG. 3.

Particles of an opaque material 5 such as carbon or graphite with the size of 20 - 60 millimicrons are sprayed uniformly over the photosensitive layer 2a. Those of the particles on the light-exposed portions 4 are removed by the well-known method such as air blast or immersion in a solvent. Although the need of this process may seem to be eliminated by the later-described process of washing, the removal of the particles as mentioned above is desirable to assure successful results of the washing process. Thus, the light-exposed portions 4 are rendered light-transmissible and a layer of the opaque material 5 is formed on the photo-

sensitive layer 2a except on the light-exposed portions 4, thereby forming in the photosensitive sheet 21 a light-transmissible portion of a smaller diameter than the opening 1c of the shadow mask 1. Subsequently, the photosensitive sheet 21 should be washed with a detergent solution containing an anionic surfactant such as an alkali salt of higher fatty acid, alkyl sulfate, alkylaryl sulfonate, or sulfosuccinic acid ester so that the light-exposed portions are melted off thereby to clearly define the boundaries for the light-transmissible portion or to produce a well-shaped light-transmissible hole.

In an example, a photosensitive layer 2a consisting of viscous natural rubber and having a thickness of 1 micron is exposed to light from a mercury lamp of 400 W located 30 cm away through shadow mask openings having a diameter of 0.32 mm and through a transparent layer 2b having a thickness of 8 microns to form light-exposed portions in the photosensitive layer 2a, and then carbon particles of 20 millimicrons are sprayed on the photosensitive layer 2a. The photosensitive layer 2a is processed with an air blast in order to remove particles on the light-exposed portions no longer having viscosity and then is washed by the immersion thereof in a 0.5 percent aqueous solution of sodium alkylbenzenesulfonate for 30 minutes. During the washing process, attention should be paid so as not to subject the inner side of the shadow mask assembly to the detergent solution, because otherwise the close contact between the shadow mask and the transparent sheet may be lost. In this way, the light-transmissible holes 4 having a diameter of 0.23 mm are obtained. In addition to the above-mentioned immersion, spraying may be employed to wash away the light-exposed portions of the photosensitive layer with a detergent solution, also paying attention as above mentioned.

The photosensitive layer 2a may consist of such a material as polyvinyl carbazole so that electric charges in the light-exposed portions 4 are removed by exposure to light for the repulsion of the opaque material. An exposure process to form a phosphor screen is followed through the shadow mask 11 having the photosensitive sheet 21 i. e., through the shadow mask assembly. In the above-mentioned method, a panel for the cathode-ray tube with phosphor dots smaller in diameter than the opening of the shadow mask is obtained much more easily than the conventional method employing post-etching. Upon completion of the exposure process, the photosensitive sheet 21 fixed at the side face of the frame 3 is easily removed to recover a desired shadow mask 1.

In addition to a color cathode-ray tube of shadow mask type referred to above, the present invention is easily applicable to a color cathode-ray tube of chromatron type.

As is apparent from the foregoing detailed description, in the present invention a transparent sheet is put over a shadow mask to make the size of the light-

transmissible portion smaller than that of the shadow mask opening and at least the photosensitive layer is washed thereby to form a light-transmissible hole in the photosensitive layer. Unlike the conventional methods, the present invention has the advantages that no special measures are required to prevent partial corrosion of the shadow mask and to maintain the diameter of the opening thereof. In particular, the process of washing the photosensitive layer with a detergent solution contributes to the clarification of the boundaries for improved dimensional accuracy for the light-transmissible holes in the photosensitive layer. Furthermore, the method of the invention has the advantage of the ease with which the phosphor screen is produced economically with very few substandard products.

What is claimed is:

1. In a method for making a phosphor screen of cathode-ray tube comprising the steps of providing a transparent layer on that surface of a shadow mask which faces the phosphor screen within said cathode-ray tube, said shadow mask being carried by a supporting frame, said transparent layer being capable of attenuating light passing therethrough, providing a photosensitive layer on said transparent layer said photosensitive layer upon exposure to light being removable by washing with a detergent solution, exposing said photosensitive layer to light through said shadow mask and transparent layer to form light-exposed portions smaller in diameter than the shadow mask openings in said photosensitive layer, developing said photosensitive layer with a light absorbing material that adheres to the unexposed portions to form, in accordance with the shadow mask openings, a pattern of effective light-transmissible holes in said photosensitive layer thereby obtaining a shadow mask assembly, and forming a pattern of phosphors using said shadow mask assembly, the improvement comprising the fact that prior to the formation of the phosphor pattern, said shadow mask assembly is washed with a detergent solution to remove said light-exposed portions of said photosensitive layer.

2. The method according to claim 1, in which said detergent solution includes an anionic surfactant.

3. The method according to claim 1, in which said anionic surfactant is selected from the group consisting of alkali salt of higher fatty acid, alkyl sulfate, alkylaryl sulfonate, alkyl sulfonate and sulfosuccinic acid ester.

4. The method according to claim 1, in which said transparent and photosensitive layers are fixed at those portions which do not contribute to the formation of said phosphor pattern.

5. The method according to claim 1, in which said photosensitive layer includes a material capable of photopolymerization and said exposing step is carried out at a temperature within a range from room temperature to 90°C.

\* \* \* \* \*